

## UNITED STATES PATENT OFFICE.

ADOLPH SCHWENTERLEY, OF BROOKLYN, NEW YORK.

## ROTOGRAVURE INK.

No Drawing.

Application filed August 14, 1922. Serial No. 581,882.

*To all whom it may concern:*

Be it known that I, ADOLPH SCHWENTERLEY, a citizen of the United States, residing in Brooklyn, county of Kings, and State 5 of New York, have invented certain new and useful Improvements in Rotogravure Inks, of which the following is a specification.

My invention relates more particularly to 10 printing inks adapted for rotogravure press work.

To be adapted for the so-called rotogravure high-speed process, an ink must be free-flowing, yet it must cover well and dry 15 very rapidly in order to prevent setting off of the ink on contiguous folded sheets, particularly in newspaper work. To provide a free flowing rapid drying ink of this character, it has been common to avoid the use 20 of the customary vehicle of boiled linseed oil, and substitutes of the same general characteristics, and to employ naphtha or benzol in conjunction with a material or materials which will give it body while not 25 materially reducing its volatility and hence its agency in effecting rapid drying. Gum mastic and other gums and resins have been used as this body material. Inks composed of naphtha and gum as the primary vehicle, 30 and colors in oil, have been satisfactory from the standpoint of reproduction, but have been found to be objectionable from two standpoints: First, because of the inflammability of the ink and its fumes, and 35 secondly because of the toxic effect of the fumes upon the pressmen.

The primary object of the invention is to provide an ink of this class which will be non-inflammable or substantially non-inflammable. A subordinate object is to provide such an ink which will be substantially free from toxic influences. I have discovered that certain chlorine-hydrocarbon derivatives, which have heretofore been 45 recognized only as powerful non-inflammable solvents, are capable of being successfully compounded with ingredients of the ink so as to impart the characteristic of non-inflammability to the ink as a whole 50 without causing undue penetration of the paper by the ink or lateral spreading thereof. On the contrary, I am able to produce a sharpness which has heretofore not been achieved with rotogravure inks.

55 Of the group of chlorine-hydrocarbon derivatives, I prefer carbon tetrachloride or

tetrachlorethane, although the other chlorine derivatives of ethane—dichlorethylene, trichlorethylene, perchlorethylene and pentachlorethane, may be regarded as equivalents, for example. All of these are of excessive volatility. For instance, an ink comprising a vehicle of carbon-tetrachloride of uncontrolled volatility, mixed with such body-material as gum-mastic or gilsonite, 60 will render the printing plates useless by dense deposits within the engraved lines, by reason of undue surface volatilization, even where, as in the rotogravure process, the time for this is very limited due to passing the plates directly into the fountain and then to a wiper to remove excess of ink. 70

With due provision for controlling the volatility of such a chlorine-hydrocarbon derivative, it may be used as the only solvent. I have discovered however, that such controlling ingredient can be part of the solvent. Thus, a less complex hydrocarbon body, such as naphtha, will provide this 75 control and form part of the solvent, without use in such large proportion as to make the ink inflammable as a whole. As equivalents of naphtha for such purpose may be mentioned benzol, commercial benzine, turpentine, and other hydrocarbons, preferably 80 non-fatty. Also, such solvents as these reduce the cost of the ink as compared with ink having carbon tetrachloride or its equivalent as the entire solvent. 85

I employ such proportion of pigment and 90 vehicle ingredients as may be desired, together with a desired proportion of solvent composed partly of a substance to render the entire composition non-inflammable notwithstanding the high degree of inflammability of the other portion of the solvent. For example, carbon tetrachloride in the proportion of about  $32\frac{1}{2}$  parts by volume to 100 parts by volume of gasolene or the like. Or, if desired, the carbon tetrachloride 100 may displace the gasolene to a greater extent, and in such case the ink will dry with greater rapidity.

The carbon tetrachloride or its equivalent is mixed with the other ingredients in the 105 usual manner, and the entire composition ground or otherwise treated to incorporate the pigment or pigments with the vehicle and solvent, as is well known in ink manufacture. Or the proportion of carbon tetrachloride may be added to the completely 110 ground or otherwise thoroughly mixed com-

position, first prepared with a deficiency of volatile solvent of an inflammable nature such that when the volatile solvent, carbon-tetrachloride, is added, the correct fluidity of 5 the ink for rotogravure printing will be attained. However, it is preferable to render the mass non-inflammable prior to the grinding or other mixing operation, by preparing the solvent of the inflammable and 10 non-inflammable ingredients prior to mixing. Or the non-inflammable solvent may be added to the other ingredients, except the inflammable solvent, the grinding or other mixing operation then being performed, and afterward the inflammable solvent added. If carbon-tetrachloride makes 15 up the entire solvent ingredient, it of course may be mixed with the other ingredients prior to the grinding or other incorporating 20 operation.

It will be understood that costs of the ingredients may dictate one of the other orders of procedure, or the nature of the ingredient added to reduce or eliminate the inflammability may influence this.

The toxic effect of the chlorine-hydrocarbon derivatives above set forth is due to the presence of chloroform and other highly volatile substances which may be driven off 25 by heat. For example, by rapidly flowing carbon tetrachloride through a vented tube subjected to approximately 77° C. and thence into a closed container, I have succeeded in driving off the toxic constituents 30 in such measure that in use the vapors from the ink, in which the treated carbon tetrachloride forms an ingredient, are unobjectionable, having no noticeable effect upon the pressmen. The loss by such treatment is 35 less than 10% of the carbon tetrachloride.

Having described my invention, what I claim is as follows, it being understood that I claim full right to the use of equivalents for the substances named:

- 5 1. A rotogravure ink comprising a solvent mixture of inflammable liquid and a substance rendering the solvent non-inflammable.
2. A rotogravure ink comprising a solvent mixture of a petroleum product and a substance rendering the solvent non-inflammable.
3. A rotogravure ink comprising a solvent

mixture of inflammable liquid and carbon tetrachloride.

4. A rotogravure ink comprising a solvent mixture of a petroleum product and carbon tetrachloride.

5. A rotogravure ink comprising a solvent made up of inflammable liquid about 100 60 parts by volume and a substance rendering said solvent non-inflammable about 32 $\frac{2}{3}$  parts by volume.

6. A rotogravure ink comprising a solvent made up of a petroleum product about 100 65 parts by volume and carbon tetrachloride about 32 $\frac{2}{3}$  parts by volume.

7. A rotogravure ink comprising a non-inflammable solvent of such volatility and in such proportion as to impart to the ink 70 its free flowing and rapid drying characteristics.

8. A rotogravure ink comprising a non-inflammable solvent of excessive volatility, and an ingredient to control the volatility of 75 said non-inflammable solvent.

9. A rotogravure ink comprising a non-inflammable solvent of excessive volatility, and a solvent of less volatility to control the volatility of said non-inflammable solvent. 80

10. A rotogravure ink comprising a mixture of solvents, one of which is non-inflammable but of excessive volatility, and the other of which controls the volatility of the non-inflammable solvent in such degree 85 as to impart to the ink the requisite free flowing and rapid drying characteristics without rendering the ink inflammable as a whole.

11. The process of making rotogravure 90 ink consisting of rapidly flowing a chlorine-hydrocarbon derivative past a vent under a temperature adapted to drive off through the vent a substantial proportion of the toxic content, and mixing the thus treated substance, as a solvent, with ink ingredients comprising inflammable substances, whereby the ink produced is of reduced inflammability and reduced toxic effect.

In testimony whereof, I have signed my 100 name to this specification in the presence of two subscribing witnesses.

ADOLPH SCHWENTERLEY.

Witnesses:

W. LEE HELMS,  
F. H. LOGAN,